

July 11, 1961

R. S. GOY

2,992,150

CORE-SPUN YARN REINFORCED COMPOSITE PRODUCTS

Filed Oct. 2, 1956



Fig. 2.

INVENTOR.  
RONALD STANSFIELD GOY  
BY *Benj. J. Rauber*  
ATTORNEY

# United States Patent Office

2,992,150

Patented July 11, 1961

1

2,992,150

## CORE-SPUN YARN REINFORCED COMPOSITE PRODUCTS

Ronald Stansfield Goy, Castle Bromwich, near Birmingham, England, assignor to Dunlop Rubber Company Limited, London County, England, a British company

Filed Oct. 2, 1956, Ser. No. 613,368

Claims priority, application Great Britain Oct. 4, 1955

4 Claims. (Cl. 154—5.2)

This invention relates to composite products containing textile yarns and plastic compositions having a basis of a polyvinyl compound.

Cotton yarns stick naturally to plastic compositions due to their fibrous nature, the hairs of the cotton staple giving in effect a mechanical lock. On the other hand continuous filament yarns made, for example, of regenerated cellulose, nylon or polyesters require to be hot-stretched to avoid subsequent deformation and then have to be treated with a bonding agent in order to make them adhere satisfactorily.

Artificial staple fibre yarns are produced from rayon, nylon or like material by cutting filaments thereof into staple form and spinning the staple fibre thus formed. Such yarns can also be used as a reinforcement but they are generally not so strong as and have a higher extensibility than comparable yarns made of continuous filaments. Moreover it has been found that the force necessary to break down the adhesion between the yarn and the composition is normally proportional to the strength of the individual fibres forming the yarn and therefore with the weaker or staple fibres, e.g. rayon, adhesion is less satisfactory than with the stronger fibres e.g. nylon.

It has now been found that if continuous filaments and staple fibres are spun together by the process known as core-spinning or "Belgian doubling," the continuous filaments being used in a proportion of from 50% to 90% by weight, yarn may be produced which will adhere better to plastic compositions having a basis of polyvinyl compound than yarn formed solely of continuous filaments and which still possesses a satisfactory tenacity. Moreover the tenacity of the core-spun yarn is found to be approximately equal to the sum of the tenacities of yarns obtained by spinning each of the components separately.

According to the present invention therefore a composite material comprises core-spun yarns comprising continuous filamentary material twisted together with staple fibres, the proportion of continuous filamentary material being between 50% and 90% by weight, embedded in a plastic composition having a basis of a polyvinyl compound.

The construction of the core of spun yarn and of a belting embedding it are shown in the accompanying drawings in which

FIG. 1 is a side view of a portion of the yarn, a part of the outer spun yarn being shown as removed at one end to show the structure of the core, and

FIG. 2 is a cross-section of a rubber belting showing the position of the yarn or thread either as separate longitudinally extending threads or as a fabric having such threads as warp and light weft.

In the core of spun yarn of FIG. 1 the core 10 is made of a number of filaments 11 having a twist and extending longitudinally of the yarn. These filaments are of continuous filamentary material. Spun on this core is a layer of staple fibres 12.

In the section of FIG. 2 cords 13 of the type illustrated in FIG. 1 are embedded in a mass 14 of the plastic composition. The cords 13 may be in the form of longitudinally extending warp having filler threads 15.

2

The invention is of particular importance in the production of belting made of a polyvinyl chloride composition reinforced by a textile material, since it makes it possible to obtain the advantages both of continuous filament yarns and also of staple fibre yarns. Thus a yarn made by core-spinning a continuous filament nylon or Terylene yarn with cotton fibres possesses both the high tenacity of the core yarn together with the good bonding properties of cotton yarns for polyvinyl chloride compositions, so that by using such yarn conveyor or transmission belting can be obtained having the high strength obtainable with nylon or Terylene reinforcements and the good adhesion between the reinforcement and the composition obtainable with cotton or other staple fibre yarn.

Filamentary materials which may be used include those made of regenerated cellulose, nylon or the polyester sold under the registered trade mark "Terylene," and the staple fibres may be of such materials or may be natural fibres e.g. cotton.

Furthermore, the filaments and the staple fibres in a yarn may be of similar or dissimilar materials. For example rayon, nylon or "Terylene" filaments may be spun with a layer of cotton staple. Other suitable combinations are, nylon filaments and nylon staple, rayon filaments and rayon staple, "Terylene" filaments and "Terylene" staple, "Terylene" filaments and nylon staple, and nylon filaments and "Terylene" staple.

In core-spinning or "Belgian doubling" the yarn is spun on a conventional spinning frame. The staple fibre, in roving form, is drafted in the usual manner and the continuous filament yarn is fed in at the front roller and twisted with the staple. By correctly balancing the twists, a layer of staple fibre is formed round the centre core of the continuous filament. If the continuous filament is nylon then by core-spinning with a low extensibility staple fibre, e.g. cotton, the additional advantage is obtained that the extensibility and creep of the composite yarn is lowered and the necessity for hot-stretching is reduced or eliminated, the tendency towards heat shrinkage being also reduced.

Preferably the yarn comprises between 20% and 40% staple fibre though the proportions of continuous filament to staple may be varied providing the latter does not exceed 50% of the yarn. In this respect it has been found that yarns constituted by 70% "Terylene" and 30% cotton, or 60% nylon and 40% cotton provide, when doubled, satisfactory cords.

An example of suitable yarn for use in conveyor belting is as follows:

The basic yarn was made by core-spinning 250 denier Terylene with 30s cotton roving to a resultant yarn count of 12s. The core-spun yarn was then doubled twelve fold and the doubled yarn cabled four fold to give a 12s/12/4 construction.

The cabled cord had a tensile strength of 225 lb. and its composition was approximately 60% Terylene and 40% cotton.

The calculated strength of the continuous filament Terylene in the cord is 172 lb.

The cotton used was combed Egyptian Karnak of Fully Good Grade. A 30s/12/4 cord from this type of cotton should have a strength of approximately 53 lb., i.e. the difference between the strength of the blended cord and that of the calculated strength of its Terylene component.

The cord thus develops the combined strength of the two components.

The twist particulars were as follows:

70 Twist/1"—single 12.0 Z (core-spun)  
Twist/1"—first folding 5.0 S  
Twist/1"—second folding 2.0 Z

Conveyor belting fabric of the following construction was made with this cord as the warp and with a continuous filament nylon weft.

Threads/1"

Warp 13  
Weft 8

Plies:

Warp 12s/12/4  
Weft 210 denier/8/3

Weight/square yard 52.0 oz.

The finished belting fabric had a tensile strength of 2,100 lb./1" ply in the warp direction and 540 lb. per inch in the weft direction.

Belting may be made by impregnation of this fabric with a flexible polyvinyl composition consisting of:

|                    | Parts by weight |
|--------------------|-----------------|
| Polyvinyl chloride | 60              |
| Tritolyl phosphate | 20              |
| Diocyl phthalate   | 10              |
| Stabiliser         | 5               |
| Colour and fillers | 5               |

and applied to the fabric in known manner such as by spreading or by calendering on a friction calender. The coated fabric is then cut to the desired width and a number of the coated plies assembled and covers consisting of the above composition applied on each side of the impregnated fabric assemblage. The whole is pressed while under stretch at a temperature sufficient to fuse the thermoplastic polyvinyl composition. The belting is cooled down before stripping from the press.

The flexible composition employed may contain polyvinyl chloride or a copolymer of vinyl chloride with vinyl acetate and/or vinylidene chloride with a suitable plas-

30  
35

ticiser, e.g. a mixture of tritolyl phosphate and diocyl phthalate.

Having now described my invention, what I claim is:

1. A composite material comprising a plastic composition having a basis of a polyvinyl compound selected from the group consisting of polyvinyl chloride, copolymers of vinyl chloride and vinyl acetate and copolymers of vinyl chloride and vinylidene chloride having embedded therein yarns comprising a core of continuous

10 filamentary material having a layer of a roving of staple fibres spun thereon wherein the proportion of continuous filamentary material is between 50% and 90% by weight of the yarn.

2. A composite material according to claim 1 wherein the continuous filamentary material of the core-spun yarns is nylon and the staple fibres are cotton fibres.

3. A composite material according to claim 1 wherein the continuous filamentary material of the core-spun yarns is polyethylene terephthalate and the staple fibres are cotton fibres.

4. The composite material of claim 1 in which said yarns are doubled yarns each having a core of filamentary material and having a layer of a roving of staple fibres wound thereon.

#### References Cited in the file of this patent

#### UNITED STATES PATENTS

|           |                 |               |
|-----------|-----------------|---------------|
| 2,053,123 | Alles           | Sept. 1, 1936 |
| 2,411,326 | McMillin et al. | Nov. 19, 1946 |
| 2,477,652 | Robbins         | Aug. 2, 1949  |
| 2,526,523 | Weiss           | Oct. 17, 1950 |
| 2,608,874 | Waugh           | Sept. 2, 1952 |
| 2,721,158 | Mans            | Oct. 18, 1955 |
| 2,755,214 | Lyons et al.    | July 17, 1956 |